# EUROPEAN PATENT SPECIFICATION

(11) **EP 2 950 025 B1**
(45) Date of publication and mention of the grant of the patent: **21.12.2016**
(21) Application number: 15169357.9
(22) Date of filing: 27.05.2015
(51) Int. Cl.: F27D 11/12, B05D 7/14, B05D 1/18, E04C 5/01, F27D 3/12

(54) **ELECTROMAGNETIC HEATING TRANSFERRING MEANS FOR STEEL BARS BETWEEN WORKING STATIONS COMPRISING TWO DIP TANKS CONTAINING BITUMINOUS SOLUTIONS**
ELEKTROMAGNETISCHE WÄRMEÜBERTRAGUNGS-EINRICHTUNGEN FÜR STAHLSTANGEN ZWISCHEN ARBEITSSTATIONEN, UMFASSEND ZWEI TAUCHTANKS, ENTHALTEND BITUMINÖSE LÖSUNGEN
MOYENS DE TRANSFERT DE DISPOSITIFS DE CHAUFFAGE ELECTROMAGNETIQUES DE BARRES D'ACIER ENTRE DEUX STATIONS DE TRAVAIL COMPRENANT DEUX BAC D'IMMERSION CONTENANT DES SOLUTIONS BITUMINEUSES

(30) Priority: 27.05.2014 IT CT20140010
(43) Date of publication of application: 02.12.2015
(73) Proprietor: Santonocito, Antonio, 95040 Motta S. Anastasia (CT) (IT)
(72) Inventor: Santonocito, Antonio, 95040 Motta S. Anastasia (CT) (IT)
(74) Representative: Sarpi, Maurizio

(56) References cited:
- EP-A1- 2 484 841
- JP-A- 2005 231 796
- RU-C2- 2 181 174
- US-A- 3 871 533

## Description

The present disclosure relates to the building sector and more in particular to an innovative method, and the corresponding means, for coating the steel bars used in the building sector with a layer of bituminous material in order to guarantee conservation thereof over time.

Right from the very first forms, up to the present day, reinforced-concrete structures have been subject to limited duration because the steel bars are inevitably attacked by rust (iron oxide), which jeopardizes the strength and integrity of the structures and which in the majority of cases leads to the need for demolition thereof.

A large number of scientific researchers (engineers, architects, scientists, experts on building materials, etc.) throughout the world have devoted their energy over the years to seeking a solution for improving the strength and conservation over time of steel bars for reinforced-concrete structures, above all in the United States of America, where there is a prevalence of skyscrapers, and for which huge amounts of capital have been invested but without any altogether satisfactory results since steel bars resist only for a limited time, with the result that after approximately 60-100 years such buildings undergo corrosion of the steel and have to be demolished.

The limit of researchers has been to concentrate their attention and experiments exclusively on cold-dipping of the bars in one and only one first tank, thus making just one first pass for treatment of the bars.

EP-A 2484841 discloses a plant and a process for providing steel bars with a bituminous anti-oxidizing coating comprising two dipping tanks heated at different temperatures and lifting and transferring means in between.

In the Italian patent No. 1403867 filed in the name of the present applicant, a process has been described for anti-oxidizing treatment with protective baths of bituminous material of the steel bars that are used in the building sector both in load-bearing structures made of steel structural work and as skeletons resistant to bending and shear stresses of reinforced concrete.

The above process envisages a series of production steps, respectively of impregnation, where the individual bar, at ambient temperature, first comes into contact with a bath of bituminous solution at a temperature of between 6°C and 10°C, then passes to a step of first drying in air at ambient temperature, followed by a second dipping in a second tank containing a hot bituminous emulsion kept at a temperature of between 350°C and 450°C for a certain time, and eventually passes to a final drying step, where it is left to cool at ambient temperature for a time interval that varies as a function of the ambient temperature in order to obtain a metal bar that cannot be attacked by corrosion.

A task of the present invention is to rationalize the above method, rendering the process of treatment of the bars no longer dependent upon the environmental conditions and hence upon the geographical area, the season, the natural temperature gradients, etc.

Another task of the invention is to guarantee industrial reproducibility of the method, enabling control of the temperatures throughout the treatment path from the point where the steel bars are picked up to the point where they are loaded onto the conveying trolley.

The above has been obtained, according to the invention, by resorting to a thermo-electromagnetic plant, which is able to measure, adapt, and balance the various temperatures of the steel bars that are to undergo treatment with the temperatures of the antioxidant bituminous solutions contained in the dip tanks described in the aforementioned Italian patent filed in the name of the present applicant, in addition to carrying out movement of the bars through the various operating stations.

In greater detail, with the present invention:
- the first step of the treatment has been improved in so far as it has been found that it is of fundamental importance to dip the bars in a tank, appropriately built, containing a bituminous solution that is cold but at an adequate constant temperature; and
- a second step has been devised, tested, and developed, which consists in providing a second tank immediately downstream of the first, without envisaging any intermediate steps, for dipping the bars into a special hot bituminous emulsion at an adequate constant temperature.

In the course of testing, the inventors have surprisingly found that the aforesaid constant temperature is of fundamental importance, since a higher or lower temperature would not prove suitable and would nullify the result thereof.

Consequently, forming a further object of the invention is a method that envisages:
measuring the temperature of the environment in which the steel bars are deposited, the temperature of the bituminous liquid contained in the two tanks, and the temperature of the loading environment;
adapting in succession the temperature of the environment where the steel bars are located to the temperature of the bituminous liquid of the first tank, to the temperature of the bituminous liquid of the second tank, and finally to the temperature of the loading environment;
balancing the various temperatures of the steel bars and of the dipping liquid throughout the treatment path; and
articulating the steps of treatment of the steel bars from the point where they are picked up from the ground or from the furnace to the point where they are loaded onto the trolley.

Yet a further object of the invention is to provide a plant equipped with a thermo-electromagnetic device designed to carry out in succession the various treatment steps starting from measurement of the temperature of the environment in which the steel bars are deposited.

According to the invention, the above plant basically comprises a metal cage or tunnel that develops longitudinally over the entire path from outlet of the steel bars from the furnace or from where they are stored up to the final station, covering two dip tanks, contained in which is bituminous solution at different temperatures. Provided inside said cage or tunnel is a thermo-electromagnetic device constituted by a bell, closed at the bottom by an electromagnetic plate, which is slidingly guided in a suspended way along a fixed horizontal guide, via a vertical load-bearing arm. In a preferred embodiment, said electromagnetic plate defines within the bell a closed top compartment, which is used as chamber for containing equipment, and a compartment open at the bottom, which serves as chamber for heating the bars since it is able to contain the steel bars, which that, once they have been attracted by the electromagnetic plate, are carried by the bell to the various operating stations.

The temperature of the steel bars, picked up from the environment where they are deposited, must first be adapted to that of the dipping liquid of the first tank, which consists of a cold bituminous solution (6°-10°C).

Once the steel bars have come out of the first tank, their temperature must be adapted to that of the dipping liquid of the second tank, which consists of a hot bituminous emulsion (390°-410°C).

Finally, the temperature of the bars that have come out of the second tank must be adapted to that of the loading environment so that they can be loaded onto the conveying trolley.

The bell has an electromagnetic field that has the basic function of binding the two elements, namely bitumen and iron (steel bars for reinforced-concrete structures), into just one element, which becomes a single body that is compact and resistant to corrosion over time.

Further characteristics and advantages of the invention will emerge clearly from the ensuing description, with reference to the attached plates of drawings, which illustrate, purely by way of nonlimiting example, a preferred embodiment thereof.

In the plates of drawings:
Figure 1 is a top plan view of the plant;
Figure 2 is a vertical cross-sectional view according to the plane of trace A-A of Figure 1, which shows the thermo-electromagnetic bell set in a position corresponding to the first tank containing the cold bituminous solution;
Figure 3 is a vertical cross-sectional view according to the plane of trace B-B of Figure 1 of the bell in the position of Figure 2;
Figure 4 is a vertical cross-sectional view according to the plane of trace A-A of Figure 2, at a larger scale, of just the bell; and
Figure 5 is a schematic perspective view of the longitudinal cage and of the thermo-electromagnetic bell.

With reference to the figures, the plant that is described is constituted by an electromagnetic bell 12 designed to slide within a metal cage 14, which extends throughout the path for treatment of the bars 15 from the point of exit of said bars from the furnace or the point where they are picked up from the ground where they have been accumulated up to the point where they are loaded onto the trolley that conveys the treated bars, covering also two dip tanks 16, 18 that contain the bituminous solution, which are kept at a differentiated temperature by two mutually independent combustion chambers 20 and 21, respectively, set underneath said tanks.

The electromagnetic bell 12 is guided so as to slide in the cage along a horizontal load-bearing shaft or beam 24 fixed on the roof of the cage itself thanks to a vertical supporting arm 26, the bottom end of which is anchored to a magnetic plate 28, which slides downwards along two guides 30 welded to the iron pillars distributed throughout the length of the cage.

The above magnetic plate 28 separates the inside of the bell 12 into two chambers: a top chamber 32, contained in which is the equipment 34 that has the function of gradually heating the steel bars (which are located in the underlying heating chamber) to the temperature established both for the first tank and for the second tank; and a bottom or heating chamber 36, which receives the heat from the equipment of the overlying chamber and located underneath which is the magnetic plate 28, which magnetically attracts the steel bars.

The magnetic plate 28 is, in fact, subject to magnetization and demagnetization for attraction and repulsion, respectively, of the steel bars 15.

The two metal tanks 16, 18, each measuring 2.00 m x 1.00 m, are located at the base of the cage. The first contains the cold bituminous solution and the second contains the hot bituminous solution in which the steel bars are to be dipped.

The two combustion chambers are equipped, respectively, with means 42 for heating the cold bituminous solution to the temperature of 6°-10°C, and with means 44 for heating the hot bituminous emulsion to the temperature of 390°-410°C.

The plant just described enables the operations outlined in what follows to be carried out.

### Measurement of temperatures

With an appropriate distribution of temperature sensors, the temperature of the environment in which the steel bars are deposited is first measured. Then, the temperature of the bituminous dipping liquid in the first tank is measured. This is followed by measurement of the temperature of the bars after first dipping in the first tank and then measurement of the temperature of the bituminous dipping liquid in the second tank. Finally, the temperature of the loading environment is measured.

The temperature of the liquid both in the first tank and in the second tank (which is practically standard for each of the tanks) is fixed at the start of each treatment cycle (within the limits established).

### Adaptation of the temperatures

a) Adaptation of the ambient temperature of the steel bars to that of the (antioxidizing) bituminous liquid in the first tank
   The temperature of the environment in which the steel bars are deposited may vary considerably in so far as it depends upon the geographical area (in northern areas, it is approximately 15°C below zero; in southern areas, it is approximately 40°C above zero), the season, the place, the natural temperature gradients, etc. Hence, before the steel bars are dipped into the cold bituminous solution of the first tank, they must be adapted to the temperature thereof, which should be 6°-10°C.
   A difference of a few degrees centigrade (more or less, for at most 2°C) is insignificant in so far as the temperature of the bars will be regulated by the temperature of the bituminous dipping liquid.
b) Adaptation of the temperature of the bars after dipping in the liquid of the first tank (6°-10°C) to that of the (antioxidizing) bituminous liquid of the second tank (390°-410°C)
   After the steel bars have been dipped in the bituminous liquid of the first tank, they have a mean temperature of 8°C, and this temperature will have to be adapted to the mean temperature of 400°C of the liquid, i.e., the hot bituminous emulsion, of the second tank.

A difference of several degrees centigrade (more or less, for at most 10°C) is insignificant in so far as the temperature of the bars will be regulated by the temperature of the bituminous dipping liquid in the second tank.

Adaptation of the temperatures as described above is obtained via appropriate heating devices located within the so-called "equipment chamber", which gradually bring the temperature of the bars to higher values to enable dipping in the bituminous liquid of the two tanks.

When the bars are to be dipped in the bituminous liquid of the second tank, they will never have a mean temperature of 400°C but will gradually adapt to the temperature of the dipping liquid, given that iron is a conductor that immediately absorbs heat, reaching high temperatures.

Careful control of the temperatures and consequent adaptation both of the steel bars and of the bituminous dipping liquid enables the bars to blend with the hot bituminous liquid in an optimal way as compared to a simple or normal dipping.

Considering the dimensions of a tank with a width of 1.00 m and a length of 2.00 m, this will be able to contain twenty-four steel bars with a total weight of 120 kg.

### Balancing of the temperature variations

The electromagnetic field produced by the bell has the function of:
a) balancing the variations of temperature throughout the treatment path from the point where the steel bars are picked up from the ground or from the furnace to the point where they are loaded onto the trolley so that they will not undergo alterations such as scaling, air bubbles, or pitting in which a gap is created that does not enable the bituminous liquid to adhere, and consequently the bars will be subject to deterioration and hence be unusable;
b) binding the hot bituminous emulsion at the mean temperature of 400°C to the steel bars at the same temperature at the moment of dipping using the magnetic plate in such a way that the two elements, namely, bitumen and iron (steel bars), combine to form just one element, thus constituting a single body that is compact and resistant to corrosion over time; the electromagnetic field of the bell does not act on the hot bituminous liquid, but acts directly and specifically on the steel bars in so far as it causes an increase in the attractive energy of the steel bars so as to get the bitumen to penetrate therein or, rather, to get the element iron to bind with the element bitumen, it being at the same time important to bear in mind that bitumen does not penetrate in depth or, rather, into the central care of the steel bar; and
c) magnetizing and demagnetizing the magnetic plate to enable attraction and repulsion, respectively, of the steel bars and passage thereof through the four process steps.

In conclusion, the electromagnetic bell hence has the function of measuring, adapting, and balancing the variations of the temperatures of the steel bars throughout the processing cycle and of the bituminous liquid of the two tanks, which constitutes the basic premise for creating a protection for the bars such as to render them corrosion-resistant; i.e., they cannot be attacked by rust and are indestructible over time.

The bell, with all its articulated passes, is basically the device that enables blending of the two elements, bitumen and iron, into just one.

### Steps of treatment of the steel bars

Control of the temperatures must be carried out throughout the treatment path from the point where the steel bars are picked up from the ground or from the furnace to the point where they are loaded onto the trolley and follows the four steps below.

### Step I

Once the steel bars have been raised from the level of the furnace or the ground to the level of the first tank, they undergo adaptation in temperature from the value of ambient temperature to the value of the mean temperature of the dipping liquid, which is 8°C.

### Step II

The steel bars are lowered right down to the bottom of the first tank so as to be entirely dipped in the cold bituminous solution (6°-10°C).

They are then raised from the bottom of the first tank to the level of the second tank.

### Step III

The steel bars are lowered right down to the bottom of the second tank. As they are lowered, they gradually undergo adaptation to the temperature of the hot bituminous emulsion (390°-410°C).

### Step IV

As the steel bars are raised from the bottom of the second tank, they gradually undergo adaptation to the ambient temperature of the loading environment, and are pushed out so as to be loaded onto the trolley and conveyed into the various workplaces, now ready to confront any temperature.

Once a first cycle of treatment of the steel bars has been completed, a subsequent new cycle automatically starts, and so forth.

The thermo-electromagnetometer may be installed in a structure additional with respect to the steel-production complex or in another place prepared for treatment of steel bars.

With the present invention, the major drawback of iron (namely, rust, i.e., iron oxide) is overcome, so that large structures, such as large public buildings, skyscrapers, bridges, viaducts, and so forth, that will be built with these new criteria will no longer have to undergo demolition within a short stretch of time (60-100 years, as occurs today) but will even last for centuries.

Rusting, in fact, in addition to jeopardizing the compressive strength of steel, causes increase in the volume thereof, which can thus cause cracking of the concrete that coats it.

It should be emphasized that, without adaptation of the temperatures of the steel bars to those of the liquid of the two tanks, the steel would undergo alterations, namely, scaling, such as to render it unusable and inefficient.

### Control of the structure of steel and concrete

It is indispensible for the heating and dipping steps to be carried out as accurately as possible, since they are determining factors in so far as they affect the structure of iron (steel bars).

Of primary importance is adaptation of the temperatures, both during the first pass and during the second pass, so that it is necessary to:
check the structure of the steel bars to verify that that they are homogeneous and are impregnated uniformly, thus preventing any sharp jumps in temperature from start to end of the treatment process;
observe the rules regarding reinforced concrete (right dosage, water-to-cement ratio, perfect packaging and compaction of the mixture); and
ensure perfect adherence of the concrete to the steel bars.

In this connection, it is to be emphasized that in a preferred embodiment the operating rules outlined below are to be followed.

The steel bars with improved adherence that come out of the furnace are made to cool naturally down to the ambient temperature Ta.

Only when the bars have reached said temperature is treatment started, i.e., dipping of the bars in the first tank, which contains the cold bituminous solution at a temperature of from 6°C to 10°C (preferably a mean temperature of 8°C) for a maximum duration of 2 minutes.

Once the temperature of the bituminous liquid to be maintained has been established, e.g. 8°C, this must remain constant throughout the treament cycle of dipping of the bars in order for them to be homogeneous.

Constant temperature is of fundamental importance from the structural standpoint of iron (steel bars) since a temperature different from the one established at the start and different during the course of treatment produces bars with different degrees of absorption, and hence not homogeneous.

Of considerable importance are also the modalities of impregnation of the bars in the liquid. Impregnation must take place in a uniform manner over all the bars: a small variation of temperature and impregnation are sufficient for there to be produced bars that are not homogeneous and uniform.

It is important to guarantee that the constancy in temperature and the uniformity of impregnation are maintained during dipping of the bars also in the second tank, which contains the hot bituminous emulsion at the temperature of 390-410°C (preferably the intermediate temperature of 400°C).

Once the temperature to be maintained for the liquid has been set (e.g. 400°C), this must remain constant during dipping of the bars for a maximum duration of 2 minutes, to prevent bars with different degrees of absorption from being obtained, as has already been said as regards the first tank.

Likewise, as in the first pass within the first tank, also in the second pass within the tank at 400°C, impregnation must take place in a uniform way.

## Claims

1. A thermo-electromagnetic plant for antioxidizing treatment of steel bars used in the building sector by means of protective baths with bituminous materials, **characterized in that** it comprises:
a metal cage or tunnel that develops longitudinally over the entire path that the steel bars follow from their exit from the furnace or from where they are stored, there being provided in said path various operating stations that comprise two consecutive dip tanks containing bituminous solution at different temperatures; and
within said cage or tunnel, a thermo-electromagnetic device constituted by a bell, closed at the bottom by an electromagnetic plate, which is slidingly guided along a fixed horizontal guide,
said electromagnetic plate defining within the bell a closed top compartment, which is used as chamber containing equipment that also has the function of gradually heating the steel bars, which, once attracted by the electromagnetic plate, are received in the open underlying compartment, which serves as heating chamber, and are then carried, having been magnetized by said bell, to the various operating stations.

2. The thermo-electromagnetic plant as per the preceding claim, **characterized in that** within said cage or tunnel the electromagnetic device is slidingly guided suspended along a horizontal guide fixed at the top to said cage via a vertical load-bearing arm.

3. The thermo-electromagnetic plant as per the preceding claims, **characterized in that** of the two metal tanks located at the base of the cage, the first one reached by the steel bars along their path within the cage or tunnel contains the cold bituminous solution and the second tank contains the hot bituminous emulsion,
underneath the two metal tanks there being provided two combustion chambers, the first of which is equipped with means for heating the cold bituminous solution to the temperature of 6°-10°C, and the second is equipped with means for heating the hot bituminous emulsion to the temperature of 390°-410°C.

## Patentansprüche

1. Thermoelektromagnetische Anlage zur antioxidativen Behandlung von im Bausektor verwendeten Stahlstäben mittels Schutzbädern mit bituminösen Stoffen, **dadurch gekennzeichnet, dass** sie Folgendes umfasst:
einen Metallkäfig oder -tunnel, der sich in Längsrichtung entlang des gesamten Weges erstreckt, dem die Stahlstäbe von ihrem Austritt aus dem Hochofen oder von dort, wo sie gelagert werden, folgen, wobei in dem Weg verschiedene Bearbeitungsstationen vorgesehen sind, die zwei aufeinanderfolgende Tauchbecken umfassen, die eine bituminöse Lösung mit unterschiedlichen Temperaturen enthalten; und
im Inneren des Käfigs oder Tunnels eine thermoelektromagnetische Vorrichtung, die durch eine Glocke gebildet ist, die am Boden durch eine elektromagnetische Platte verschlossen ist, die gleitend entlang einer feststehenden horizontalen Führung geführt wird,
wobei die elektromagnetische Platte mit der Glocke eine geschlossene obere Abteilung definiert, die als Kammer verwendet wird, die Einrichtungen enthält, die auch die Funktion haben, die Stahlstäbe allmählich zu erwärmen, die, nachdem sie durch die elektromagnetische Platte angezogen wurden, in der offenen darunterliegenden Abteilung aufgenommen werden, die als Erwärmungskammer dient, und die, nachdem sie durch die Glocke magnetisiert wurden, zu den verschiedenen Bearbeitungsstationen befördert werden.

2. Thermoelektromagnetische Anlage nach dem vorhergehenden Anspruch, **dadurch gekennzeichnet, dass** die elektromagnetische Vorrichtung im Inneren des Käfigs oder Tunnels gleitend und an einem vertikalen lasttragenden Arm aufgehängt entlang einer an der Oberseite des Käfigs befestigten horizontalen Führung geführt wird.

3. Thermoelektromagnetische Anlage nach den vorhergehenden Ansprüchen, **dadurch gekennzeichnet, dass** von den zwei Metallbecken, die an der Basis des Käfigs angeordnet sind, das erste, das von den Stahlstäben entlang ihres Wegs im Inneren des Käfigs oder Tunnels erreicht wird, kalte bituminöse Lösung enthält und das zweite Becken heiße bituminöse Emulsion enthält,
wobei unterhalb der zwei Metallbecken zwei Verbrennungskammern vorgesehen sind, von denen die erste mit Mitteln zum Erwärmen der kalten bituminösen Lösung auf eine Temperatur von 6° bis 10°C versehen ist und die zweite mit Mitteln zum Erwärmen der heißen bituminösen Emulsion auf eine Temperatur von 390° bis 410°C versehen ist.

## Revendications

1. Installation thermo-électromagnétique pour le traitement d'anti-oxydation de barres en acier utilisées dans le secteur du bâtiment au moyen de bains de protection avec des matières bitumineuses, **caractérisée en ce qu'**elle comprend :
une cage ou un tunnel métallique qui s'étend longitudinalement sur tout le trajet que les barres en acier suivent de leur sortie du four ou de là où elles sont stockées, étant prévues sur ledit trajet diverses stations opérationnelles qui comprennent deux cuves d'immersion consécutives contenant une solution bitumineuse à différentes températures ; et
dans ladite cage ou ledit tunnel, un dispositif thermo-électromagnétique constitué par une cloche, fermée vers le bas par une plaque électromagnétique, qui est guidée de manière coulissante le long d'un guide horizontal fixe,
ladite plaque électromagnétique définissant à l'intérieur de la cloche un compartiment supérieur fermé, qui est utilisé comme une chambre contenant des équipements qui ont également pour fonction de chauffer progressivement les barres en acier qui, une fois attirées par la plaque électromagnétique, sont reçues dans le compartiment sous-jacent ouvert, qui sert de chambre de chauffage, et sont ensuite transportées, ayant été magnétisées par ladite cloche, vers les diverses stations opérationnelles.

2. Installation thermo-électromagnétique selon la revendication précédente, **caractérisée en ce que**, à l'intérieur de ladite cage ou dudit tunnel, le dispositif électromagnétique est guidé suspendu de manière coulissante le long d'un guide horizontal fixé au sommet à ladite cage par l'intermédiaire d'un bras de charge vertical.

3. Installation thermo-électromagnétique selon les revendications précédentes, **caractérisée en ce que**, parmi les deux cuves métalliques situées à la base de la cage, la première atteinte par les barres en acier le long de leur trajet à l'intérieur de la cage ou du tunnel contient la solution bitumineuse froide et la deuxième cuve contient l'émulsion bitumineuse chaude,
au-dessous des deux cuves métalliques étant disposées deux chambres de combustion, dont la première est équipée de moyens pour chauffer la solution bitumineuse froide à la température de 6°-10°C et la deuxième est équipée de moyens pour le chauffage de l'émulsion bitumineuse chaude à la température de 390°-410°C.
